

J. E. BUCHER.

METALLURGICAL AND CHEMICAL PROCESS.

APPLICATION FILED APR. 15, 1912.

1,087,900.

Patented Feb. 17, 1914.



Inventor  
John E. Bucher  
By his Attorney  
Rosenbaum & Stockbridge.

# UNITED STATES PATENT OFFICE

JOHN E. BUCHER, OF COVENTRY, RHODE ISLAND, ASSIGNOR TO NITROGEN PRODUCTS COMPANY, A CORPORATION OF RHODE ISLAND.

## METALLURGICAL AND CHEMICAL PROCESS.

1,087,900.

Specification of Letters Patent.

Patented Feb. 17, 1914.

Application filed April 15, 1912. Serial No. 690,886.

*To all whom it may concern:*

Be it known that I, JOHN E. BUCHER, a citizen of the United States, residing at Coventry, in the county of Kent and State 5 of Rhode Island, have invented certain new and useful Improvements in Metallurgical and Chemical Processes, of which the following is a full, clear, and exact description.

This invention relates to a novel process 10 of manufacture, one aspect of which pertains to the purification of metals generally, and more particularly iron, with the formation of other commercially valuable products and by-products incident thereto.

With the exception of aluminum, iron is 15 probably the most abundant metal in the earth, but its important ores are nearly all oxygen compounds. In practice it is nearly always obtained by reducing these ores with 20 carbon in a blast furnace, or the like. The crude iron thus obtained, known in the art as pig-iron, is very impure and frequently contains only about ninety-two per cent. of 25 iron. The impurities in the pig-iron consist 30 of variable quantities of carbon, silicon, phosphorus, sulfur, manganese, slag, occluded gases, and other substances. These impurities come partly from the ore and partly from the materials used in the manu- 35 facture of the iron. During the past hundred years considerable progress has been made in the removal of these impurities, but notwithstanding these advances in the art, really pure iron is not yet prepared on 40 a large commercial scale. This is due partly to the difficulty or expense of removing certain constituents from the iron. The processes of purification, which are now in use, such as the Bessemer, basic Bessemer, basic 45 open-hearth, acid open-hearth, and puddling, practically all depend on oxidation; the oxygen being usually obtained from the air or from iron ore ( $Fe_2O_3$ ) or its equivalent, or from air and oxid; and in substance- 50 tially all of these processes, oxygen is the active element used in the purification, and the elements carbon, silicon, manganese, sulfur and phosphorus are oxidized and thus eliminated in the escaping gases, or else in 55 the form of slags. These processes, while serving admirably in many respects are attended with many serious disadvantages; such as requiring the ores, the metal treat- 60 ed, and the furnace linings, and the like, to be of certain compositions in many cases. 55 As the degree of oxidation must necessarily be limited in most, if not all of the methods used at present, for economic and other considerations, the removal of the impurities is practically never complete; and in some 60 cases these methods even result in entire failure to remove the most objectionable impurities. Slags are formed and these sometimes interfere with the process. In some cases, excessive loss of metal or time is involved. In certain processes the energetic 65 oxidation causes serious injury to the metal and thus necessitates the use of deoxidizing agents such as manganese or silicon. Indeed, it sometimes becomes necessary to add 70 somewhat expensive alloys or materials containing such elements as manganese or silicon, in order to maintain the required high 75 temperature during the process of oxidation. When air, which contains only about one 80 volume of oxygen to four volumes of nitrogen, is used as the source of oxygen, an enormous volume of inert nitrogen is carried along with the oxygen necessary for the process. The large volume of inert gas 85 thus introduced into a given process necessitates the use of extensive pumping machinery and unduly large furnaces and converters. The nitrogen, which in such processes is useless, is raised to a high tempera- 90 ture during the purification operations, which causes an excessive loss or waste of heat. For example, in the Bessemer process roughly about seventy-five per cent. of the heat produced by the combustion of car- 95 bon to carbon monoxide is lost on account of the waste nitrogen. My process practically eliminates this waste of energy and contem- 100 plates in its preferred form heating the metal or material which is to be treated or purified, *i. e.* iron, with a mixture (or compound) comprising nitrogen (or a nitrogenous compound) and one or more powerful reducing elements, such for example as the metals of the alkali or alkaline earth groups; or compounds of such elements. In other words, I may use a mixture comprising nitrogen and one or more of these reducing elements, *e. g.* sodium and magnesium; or I may use a compound of nitrogen and one or more of these elements, *e. g.*

magnesium nitrid; or a nitrogenous compound and one or more of these reducing elements; etc.

My invention also contemplates the use in the process when desired of alloys containing a powerful reducing element or elements.

Sodium and potassium are particularly well adapted for my novel process on account of their chemical activity and volatility; while sodium has the added advantage of cheapness. While these recited elements are preferred, I do not desire, however, to be limited thereto in any sense, since any suitable material which may be characterized as a powerful reducing agent, or element, is regarded as within the purview of my invention.

The relative proportions of the elements used in the process may be widely varied, and depend upon the nature of the impurities present in the substance treated, and the extent to which it is desired to remove these impurities. Assuming that sodium be the metal used, by way of illustration, so little thereof may be involved in the process, in some cases, that the mixture, for example, with nitrogen, may comprise but a trace of the sodium. Indeed, in some cases the nitrogen may be used alone. This aspect of the invention is distinguished from the usual processes, in that, in such case, the nitrogen is the active purifying agent, in contradistinction to oxygen. In other cases it will sometimes be desirable to use so little nitrogenous matter that the reagents will consist substantially of, for example, alkali or alkaline earth metals. It will be understood, however, that while the sodium, for example, may have independent functions or actions of its own; and in like manner the nitrogen may have independent functions, there is yet a peculiar relationship between such elements whereby they conjointly serve to effect decarburization of the material treated. Considered from this point of view, therefore, the process, in so far as it relates to the decarburization of iron, for example, is practically independent of the separate and independent functions of the reducing element or elements, and the nitrogen; and while it is almost inevitable that such individual constituent elements will act to some measure, in any case independently, such action is incidental and unavoidable to their combined action. The claims herein accordingly do not attempt to cover these separate and independent actions of the elements employed, specifically.

As above indicated, instead of using free metals of, for example, the alkali or alkaline earth groups, some of their compounds which are reactive in my process and which will furnish in such case an alkali or alkaline earth metal, and in some cases a certain amount of nitrogen in addition, for example,

may be used. Cyanamids, such as disodiuni cyanamid, and amids, such as sodium amid, etc., are among the compounds of this type which may be used in the process. The nitrogen used in my process may also be obtained from such nitrogenous compounds as ammonia, nitrids, and the like, or mixtures of such substances; and it may be, and in many cases preferably is, free nitrogen. If nitrids are used they may, if desired, be produced from nitrogen by the addition of nitrid forming elements to the metal or substance which is to be treated.

When air is injected into molten iron, as in known processes, the oxygen is so much more active than the nitrogen that the latter is practically inert; as it is generally considered. It is, hence, desirable in most cases, when conducting my novel process, to exclude air. It is also desirable usually to, as far as practicable, exclude water and water-forming constituents from participation in the reactions involved in the process. A certain amount of these may be unavoidably present in the substance to be treated or purified, but such cannot in many cases be helped; and all that can be done is to avoid the wilful introduction of such compounds as hydrates, for example, which contain certain water forming constituents.

The above statements conclusively show that the principles of my process for the purification of iron, and especially for the decarburization thereof, are distinctively different from those of the present commercial processes. These known processes, considered as a whole, are oxidation processes, and they depend upon oxygen for the active element, in the purification. On the other hand my process is a reduction process which makes use of nitrogen alone in certain aspects of the same, and of powerful reducing elements, such as the alkali or alkaline earth metals, in other aspects of the same, and yet further, of a combination of nitrogen or nitrogenous matter and such reducing elements, the latter more particularly for decarburization purposes. This distinction is fundamental, as even the basic processes which are now in commercial use are really strictly oxidation processes in which basic material is used primarily to remove the phosphorus.

In my process free nitrogen, which, in the present commercial processes which use oxygen of the air, is an undesirable inert element which cannot conveniently be avoided, not only becomes an active participant in the reactions involved; but further, becomes fixed and absorbed more or less completely to form nitrogenous compounds such, for example, as cyanogen compounds or nitrids. On account of these radical differences my process overcomes very many of the disadvantages of those heretofore in use.

for purifying iron and the like, and it also has many other and even more novel advantages. For example: it not only allows the fixation of atmospheric nitrogen with 5 the production of cyanogen compounds or nitrids, as above stated; but, further, it facilitates the production of ammonia, and similar compounds; while it effects a saving of the carbon present in the mass to be 10 treated. Thus instead of oxidation products, such as carbon monoxid, carbon dioxid, or carbonates, I obtain cyanid, for example. This latter production may be represented by the equations:



These reactions are strongly exothermic; 20 and therefore may furnish a new means of getting the high temperature necessary in a modified Bessemer or similar process.

Owing to the fact that it is unnecessary in my process to heat up a relatively enormous bulk of inert nitrogen, and owing to the 25 powerful exothermic reactions involved, it should become possible for heating purposes, to utilize the carbon, present in the charge, much more advantageously than in many 30 known processes. My experiments have demonstrated that it is possible to augment this heating effect by the addition of carbon; while the heating effect will still further be intensified by introducing sodium or other 35 suitable reducing metal in the form of a vapor, either alone, or in a hot gaseous or vaporous blast. This blast, for example, may consist of hot nitrogen and sodium vapor. I am of the opinion that this will do away with the 40 necessity for using iron rich in silicon and manganese, in the Bessemer process, and of metals rich in phosphorus and low in silicon for the basic Bessemer process. This should be of great value because the Bessemer processes 45 are very exacting, in that they require definite composition in the iron ores used for the preparation of the metal. These ores are expensive, and the herein described process will hence probably enable the use 50 of cheaper ores.

Carbon in any form, even as graphite, or as carbids, *e. g.* iron carbid, may be readily and completely removed from iron by my process; or it may be removed to substantially any desired extent. Carbon or graphitized carbon may also be removed from a mixture of powdered or otherwise finely divided iron and carbon by this method. As to just what reactions and inter-reactions take place resulting in the carbon present, from whatever source, uniting with the nitrogen to form the radical CN, I am unable to positively state. Apparently, 60 an iron carbid, or, in some cases, a solution 65 of carbon in iron, is first formed, which

carbid, or solution, together with the iron carbid already present, if any, then reacts with nitrogen and sodium, or like metal or element present which is capable of forming the base of a cyanogen compound which 70 is stable at the temperature of the operation and substantially pure metallic iron is produced. The solution of carbon in iron may, of course, be either in solid or molten form. The foregoing, however, is merely my 75 theory, and I do not wish to be limited thereto in any way. The removal of graphitic carbon is of especial importance in that the presence of this substance in iron materially impairs its strength. It may here be noted 80 also that I find that carbon in other forms *e. g.* silicon carbid may be successfully removed by my process. Indeed not only is the carbon of such a compound removed, but the silicon itself is also eliminated from the 85 metal treated.

Phosphorus in steel causes brittleness under shock and general cold shortness. It has also been shown that even .005 per cent. increase in phosphorus decreases the wearing qualities of the cutting edges of tools to a sensible extent; and in general, the presence of relatively minute quantities of this impurity seriously impairs some of the most valuable characteristics of iron or 90 steel. Phosphorus is not removed to any extent by "acid" oxidation processes because the phosphorus pentoxid formed is again reduced, thus re-phosphorizing the iron. It has therefore heretofore been necessary to 95 employ basic processes, such as the basic open-hearth, or basic Bessemer, which are usually more troublesome, and in some cases, more expensive than the ordinary Bessemer process. The basic Bessemer process requires high phosphorus and low silicon on 100 account of the basic lining, and further on account of the desirability of producing a high temperature and a slag rich in calcium phosphate. In my process, the phosphorus, so far as I have been able to ascertain, is completely removed, presumably in the form of 110 a phosphid, and as the temperature can be maintained by the formation of cyanids from carbon, there is no need of a definite 115 composition of the iron used in the process. The basic Bessemer process was invented especially to remove phosphorus, and I am of the opinion that my herein described process may afford a substitute for it. 120

Sulfur is perhaps the most injurious impurity found in iron, and, to the best of my knowledge, no completely satisfactory commercial method for its removal has been found. In some cases the percentage of 125 sulfur in the metal is even increased during the effectuation of known processes. This obstacle prevents the use of certain cheap iron ores, which contain too much sulfur, in the blast furnace. In my process the sul- 130

fur is removed, presumably as sulfid. If sodium be the metal used, the following equation would represent the reaction:



- 5 As this reaction is also powerfully exothermic, the sulfur is removed very energetically and completely. This action is hence of very great importance, since sulfur in steel causes red shortness, interferes with welding, and, therefore, may cause imperfections in apparently sound castings. I am also of the opinion that sulfur and phosphorus have been the cause of many of the "mysterious" failures of structural steel, and of many serious accidents due to the breakage of railway rails; and faults due to the same cannot always be avoided, even by careful heat treatment; nor can they always be detected, even by careful tests or inspection. These facts demonstrate the value of my process wherein sulfur, phosphorus and carbon, which, so far as I am aware, cannot be removed completely by the commercial oxidation processes of today without undue loss of iron by oxidation, can be removed completely because the iron is not attacked by nitrogen, nor by the metals of, for example, the alkali or alkaline earth groups:
- In such a modified Bessemer process as I have referred to, said process would not need to be interrupted promptly at a certain time as the metal treated cannot become oxidized; so that the process could, in effect, be forced to completion without danger to the product or products. In the present Bessemer process it is commonly necessary to add ferro-manganese or similar substances to take away the excess of oxygen. In the contemplated process the current of sodium vapor and nitrogen should remove oxygen if it is present in combinations such as  $\text{FeO}$ ,  $\text{CO}$ , and similar substances, or in the form of slags. Thus it should be possible to effect a recovery of iron, instead of having to sustain a loss of about 13 to 17 per cent., as is frequently the case with the basic Bessemer process.
- I have not been able, as yet, to ascertain exactly in what order the impurities are removed from the metal to be treated, but I am of the opinion that the objectionable elements sulfur and phosphorus, are among the first to be removed, rather than among the last. If I am correct, this will result in a very great advantage, since it should not then be necessary to remove all of the carbon and then to recarburize the iron as is done in known processes.

I have above referred to the independent action of nitrogen in the process, and am of the opinion that the nitrid-forming elements, such as silicon, titanium, vanadium, and similar elements, may be removed un-

der suitable treatment, through the instrumentality of the nitrogen alone; the reactions between such elements and the nitrogen probably forming nitrids. Such nitrids may be heated with steam or with caustic alkalis, or they may be treated by other suitable methods to recover the fixed nitrogen in the form of ammonia, for example.

I have previously referred to the reduced volume of gas which might be used in such a modified Bessemer process, which should permit of the use of much smaller apparatus, such as pumping machinery, furnaces and converters, than are at present in use. This is principally due to the fact that the volume of nitrogen required to remove carbon as cyanid is only about twenty per cent. of the volume of air required in the Bessemer process to remove the carbon as carbon monoxide. This percentage may vary down to none at all in the case of operations relating to the removal of such elements as sulfur and phosphorus alone. The reduced volume of gaseous matter which would be passed through a charge would also reduce spattering of material and loss of heat.

It is also evident that my process may be used in conjunction with processes at present in commercial use, thus giving a combined oxidation-reduction process, or a combined reduction-oxidation process. Iron may also be recovered from slag, for example, by means of the herein described method; the oxids being reduced at proper temperatures. The following equations serve to illustrate this phase of my invention:



105

I consider that these reactions may be of considerable value in such a process as I have above referred to as a modified Bessemer process. The slags would be removed by the reducing action of the element or elements employed, and the freedom from slag, together with the great purity of the metal, and especially great freedom from sulfur and phosphorus should afford an ideal metal for the preparation of crucible and other fine grades of steel. High grade steel might be obtained therefrom, for example, by the addition of carbon or carbonaceous matter to the molten metal. The process may also be applied to relatively impure materials, such as metallic regulus.

In large measure, the blow holes in iron or steel are caused by carbon monoxide which is soluble in hot metal and separates partly when the metal solidifies, or which is formed by the reaction of oxids, such as  $\text{FeO}$ , in the slag with carbon. For example:



The reactions almost immediately above

100

110

115

120

125

recited will obviously prevent the formation of carbon monoxid, provided the temperature be not too high; and if such substance be present it will be reduced with production of free carbon as per the following equations:



10 I am of the opinion also that the nitrogen or nitrogen and argon current will displace or sweep out the carbon monoxid as well as other gases and volatile substances, just as such currents remove the latter substances 15 from a water solution. In this connection it should be noted that a proper effectuation of my process will afford a cheap and plentiful supply of argon, of which there is an abundance in the atmosphere, since approximately one per cent. of the latter consists of this apparently absolutely inert gas. At present practically no use is made of this element, but if it can be marketed at a low cost, undoubtedly uses will be found for it. I 20 contemplate one use of the said element in connection with the present process. I have just stated that the nitrogen, or nitrogen and argon current should displace or sweep out carbon monoxid and other gases and volatile substances from the melt, and I may here state that I contemplate in some cases using a current of substantially pure argon for this purpose. The statements in the literature indicate that the continued existence of 25 nitrogen in molten iron is very uncertain, and even should I use the current of nitrogen without any supplemental flow of relatively pure argon, I believe that the nitrogen would in probably no case be occluded in any material quantity in the molten metal. Should it be found that any appreciable quantity of nitrogen is occluded in the metal, however, it may be readily removed by the addition of nitrid forming elements. 30 It, may also, be removed by the addition of carbon with sodium or similar elements which would form cyanids according to the reaction:



50 It is obvious, of course, that this phase of my process would apply more particularly to molten metals, and especially to iron, and it may be carried out in many forms of apparatus; converters very similar to those used in the basic Bessemer process being suitable, and I have hence not attempted to illustrate apparatus wherein this phase of my process might be effectuated. It should be borne in mind, however, that in most cases air should be carefully excluded.

55 I have successfully carried out my herein described process at temperatures below the melting point of metals which are to be purified, and will now proceed to describe

with particularity the nature of the apparatus which I have used in this connection. It is to be understood, however, that the said apparatus is but one of many by means of which my process may be carried out, and I 70 hence do not desire to be limited in any particular as to either the manner or means by or in which said process may be effectuated.

75 While the particular exemplification of my process hereinafter described relates more particularly to the treatment of metals or substances at temperatures below the melting point of such substances or metals, I reiterate that I regard the treatment of metals or substances at temperatures above 80 their melting points as within the purview of my invention, and hence do not desire to be limited to operations conducted at relatively low temperatures, except where the claims specifically so state. That this contention is justified is practically proven by 85 my experiments wherein, in some cases, iron which I have treated has been formed into globules of substantially pure iron during the course of the cyanid forming operation. 90

95 Referring to the drawing which forms a part hereof and in which like reference characters designate like parts in the respective views: Figure 1 is a side elevation of an apparatus wherein my process may be carried out, one side of the muffle surrounding the retort being removed for purposes of illustration. Fig. 2 is a section of said apparatus, taken on line II—II of Fig. 1.

100 A section of heavy wrought iron pipe I is provided at either extremity thereof with a reducing cap 2, the reduced extremities of these caps being respectively connected to pipes 3 and 4, preferably of considerably 105 smaller diameter than the section 1. A T 5 is connected to the outer extremity of the small pipe or nipple 3, and a nipple 6 of the same diameter may be tapped into the opposite side of T 5. Nipple 6 is connected to a cook 7, which in turn is connected to a 110 coupling 8. The nipple or pipe section 4 is also correspondingly connected to a coupling 9. Two T's 10—10', one of which is disposed upon either side of the retort formed by the 115 tube 1 are connected respectively with the couplings 8 and 9 in any suitable manner, while a U-shaped pipe connection 11, having therein a coupling 12 and cock 13, afford a by-pass around the retort. Downwardly extending from the T 5 is a pipe 120 connection 14 having therein a cock 15 and laterally extending from the T 10' is a connection 16 in which is a cock 17. The retort 1 may be heated in any suitable manner, as by means of a series of Bunsen burners 18, 125 which for convenience may be mounted upon a common base 19 in a well known manner. A muffle or screen 20 of fire-brick, or the like, preferably having substantially the form of an inverted U, may surround the 130

retort and its burners. Suitable vents 21, for the escape of gases of combustion, and apertures 22 for the admission of air, should preferably be provided at intervals along the length of the muffle.

Assuming that iron is the metal to be treated, a suitable quantity thereof may be disposed substantially in the middle of the retort as indicated at 23. I find in practice that if the iron be finely divided, *e. g.*, pulverulent or fibrous, that the reactions are effected more rapidly than if the said metal be solid. I have successfully, however, decarburized solid masses of steel in this apparatus: the decarburization being so perfect that I have been unable to find a trace of carbon after the treatment; while I have also successfully treated pig iron herein. The metal may be introduced into the retort by unscrewing one of the reducers 2, and I similarly introduce at one end of the retort a quantity of some powerful reactive metal, *e. g.*, sodium. Nitrogen is introduced into the retort via a pipe 24, which is in communication with the T 10, upon the left hand side of the device, as shown in Fig. 1; and if the cocks 7 and 17 be opened, and cocks 13 and 15 be closed, the gaseous nitrogen will pass through the coupling 8, and connected parts, directly into the retort. Herein it is rapidly heated to a temperature preferably approximating the boiling point of sodium, if that be the reducing metal used. As the hot nitrogen passes over the sodium, designated 25, the latter vaporizes thereinto and passes together with the nitrogen through or over the metal 23 to be treated.

In the device shown, twenty burners have been somewhat diagrammatically indicated, and in practice a few of these at the extremity of the retort from which the current of nitrogen emerges are unlighted. Thus for example, fifteen gas jets may be ignited, and five burners may be left cold. As a result, the said extremity of the retort from which the nitrogen emerges is cooler than other portions of the same, and is preferably at a temperature below the boiling point of sodium, so that any sodium which passes through the mass of metal to be treated, *e. g.*, iron, will, upon entering this relatively cool end of the retort, be deposited. This procedure results in a saving of the reducing metal which accumulates in this relatively cool extremity of the retort and is there held until the current of nitrogen is reversed, in the manner hereinafter described. The nitrogen which passes through the apparatus should preferably be quite pure, with the exception, perhaps, of the argon present, and as it passes off through the cock 17 it may be collected in any suitable manner to avoid waste. After substantially all of the sodium, if sodium

be the reducing metal employed, has been transferred from one end of the retort to the other, the cocks 7 and 17 are closed and those designated 13 and 15 are opened. Thereafter the nitrogen will pass downwardly from T 10 and around a bypass 11 to T 10', and thence through the retort 1 in a reverse direction to that in which it previously flowed therethrough. It will be understood that before so reversing the current of gas the burners 18, which had previously been unlighted, are now lighted, and a corresponding number at the other extremity of the retort are turned off. As a result, the cool section or portion of the retort is transferred from one extremity of the latter to the other, so that the previously deposited sodium, for example, will be reevaporated and will again be carried through or over the metal to be treated, by the nitrogen current, to be deposited thereafter at the end of the retort from whence it originally came. The flow of nitrogen through the retort may thus be reversed at intervals until the metal to be treated has been substantially completely purified, or until all of the reducing metal has been used up. It is obvious that this metal may be introduced into the retort or vessel either in liquid or in solid form, or it may be introduced as a vapor. My experiments indicate that the higher the temperature of the operation, the more rapid the effectuation of the process. There are probably, however, limits beyond which it would be undesirable to go. In operating the apparatus herein particularly described, the temperature was maintained by means of the burners at from 700 to 800° C. I have found, however, that where the iron was in finely divided condition, and especially where additional carbon, preferably in the form of graphite, had been supplied to the mass to be treated, the reactions took place so vigorously that some of the iron was melted into globules, which would indicate that the temperature of some of the iron had been raised to the neighborhood of 1200° C., at least, and probably to 1500° C., or more. Under these last mentioned conditions the demand for nitrogen is so great that a rapid stream of the same must be flowed into the retort as the reactions tend to form a partial vacuum therein, and it is necessary in such case further to guard against a flow of gas back through the cock 17. To this end, a liquid seal 26, or the like, may be provided. With correct proportions of atmospheric nitrogen, carbon and sodium in the foregoing case, the small quantity of gas escaping through the tube 29 was practically pure argon, substantially all of the nitrogen having been greedily absorbed. Argon may only be obtained, of course, from atmospheric nitrogen, and it is assumed that this latter has been obtained

by separating it from the oxygen of the air by any suitable process, of which several commercially practicable ones are known to me. Where an excess of nitrogen passes 5 through the apparatus, it may, as I have previously stated, be collected; and may thus be used repeatedly until it has all been consumed. Should it be found in practice that any waste of sodium, for example, is 10 taking place, it is merely necessary to refrigerate, as by means, for example, of currents of air, the extremity of the retort from which the nitrogen flows, to such an extent that the temperature of the same will be 15 materially below the boiling point of the reducing metal. It may be here observed, too, that it is advantageous, in some cases, to carry out the process under a pressure considerably above atmospheric. This feature 20 is of especial advantage, for example, when the nitrogen current must be forced through the metallic mass being treated.

I have found that steel treated by the herein described process is much less rapidly 25 attacked by hydrochloric acid (20% solution) than it originally was, the steel and the iron, as it really becomes, being respectively subjected to the acid at a temperature from 80 to 90° C. In other words, 30 I have found that the practically pure iron produced by the herein described process dissolves very slowly in said acid and is far less subject to corrosion than untreated iron. It is obvious also that castings may be treated 35 in accordance with the said process so that the carbon may be taken, if desired, only from the outside thereof virtually rendering the outside of the castings malleable. When the metal treated is in solid, or relatively 40 solid form, the action seems to be that the carbon in whatever form it is present diffuses from the interior portions toward the surface of the metal, there to re-act with the nitrogen and sodium to form cyanid. 45 Iron is completely decarburized when heated to redness in an atmosphere of nitrogen and sodium vapor for a sufficient length of time, substantially pure sodium cyanid being formed. The process may even be used to 50 separate a mixture of finely divided carbon and iron in the form of filings, powder and similar states of division. When the operation is conducted at or around a red heat, the cyanid will collect upon the surface of 55 the metal treated, and can readily be obtained therefrom by lixiviation, cyanid being very soluble in water, and but a small quantity of this latter fluid therefore sufficing to expeditiously recover this valuable 60 product in the form, if desired, of a concentrated cyanid solution.

In treating solid bodies of iron such as castings, for example, obviously the carbon only at the surface of such bodies is first 65 removed, but as the process is continued it

is progressively removed from the inner portions of the castings, or the like. It is possible, therefore, to produce a material consisting of initially integrally connected layers of iron and steel, for example, which may even be alternated, since it is possible to recarburize a surface by known cementation processes. Thus, for example a block of steel may be at least partially decarburized to a given depth, of, let us say, one-half inch. Thereafter it may be recarburized by known processes to a depth of, let us say, one-quarter of an inch, and then by my herein described process a portion only of this recarburized iron may be again partially decarburized, for example, to a depth of one-eighth of an inch, and finally the surface only may be recarburized again, if desired. Again, other material than carbon may be introduced into the decarburized 80 metal. Thus vapors, for example, containing sulfur or phosphorus, or compounds thereof, or of such elements as silicon could be brought into contact with a hot surface of a metal which is to be treated, and thereby be caused to impregnate the same. 90

If finely divided iron is placed in the retort and treated in the manner above described, the product is a spongy mass, which when compressed appears as a shining or 95 highly lustrous, coherent, metallic substance which is very soft, being readily hammered or worked at ordinary temperatures. The spongy material above referred to is so readily compressed that it becomes coherent 100 and lustrous even when rubbed merely with a horn spatula, or the finger nail. Such finely divided sponge-like iron may be molded, compressed, hammered, or otherwise suitably worked, with or without the assistance of other substances, such as carbon. The objects thus formed may then be given any desired heat treatment, thus forming 105 by molding processes objects equivalent to castings, pipes, ingots, sheets and bars of 110 any desired composition.

Steel and other objects, such as sheets of metal, wire, bars, nails, or posts, may be treated by this method so as to soften or purify the surface layers alone, by selecting 115 suitable conditions in accordance with the foregoing, the surfaces to be treated being brought into contact, for example, with sodium and nitrogen, and the articles being heated for a sufficient length of time to permit of decarburization to the desired amount and depth. If desired, iron or steel objects thus treated may be given any desired subsequent mechanical or heat treatments, while retaining the core of carburized metal, to 120 give the desired rigidity and strength. The foregoing process may be continued until decarburization, dephosphorization and desulfurization, are completed depending on the rate of diffusion of such impurities 125 130

through the solid mass to be treated, at the temperature of the operation. The metal surface thus obtained is very resistant to corrosion. This phase of the process is especially adapted for the removal of impurities from sheet iron before tinning, galvanizing or sherardizing, as it removes not only the usual impurities, but also the comparatively large quantity of phosphorus which is present in the metal to prevent too great stickiness of the sheets in the rolling processes. The metal so treated is, therefore, free from the greater part of the impurities which at present cause so much corrosion of tinned iron.

The value of the herein described process will therefore be almost self-evident, and it is anticipated that it will have an important effect upon many industries. In view of the importance of the said process, and in view of the novelty residing therein, I hence desire to be limited only by the scope of the appended claims. In certain of these claims I have referred to a "process of manufacture which includes effecting a reaction," etc. Such claims I desire to be regarded as of sufficient scope to relate not only to a purified metal, *e. g.*, iron, but to other products of the treatment and of the reactions involved, *e. g.*, cyanogen compounds. It will further be understood that the word "purifying" as used herein is a general term and is intended to cover either partial or complete purification; while the term "iron" as used in the claims in connection with the said word purifying, or words of similar import, refers to wrought iron, cast iron, steel, and the like, or to alloys containing iron. In like manner the expression "changing the physical condition" of a compound is intended to cover volatilization, lixiviation, etc. Where the word "reaction" occurs in said claims, unless qualified by the adjective "direct," or the like, I intend it to be understood that such term not only includes a simple or direct reaction but a complex reaction wherein possibly several subsidiary reactions occur; this provision being obviously necessitated by the lack of exact knowledge as to just how the molecules of the several elements involved behave with respect to each other. In the appended claims the term "light metal" has been used as a generic term for such metals of relatively low specific gravity as sodium, potassium, barium, and the like. Where, also, in certain of the claims the reactions set forth involve iron or its equivalent, it is to be understood that in such case the iron may actively participate in the reaction, *i. e.* enter into or be removed from chemical compounds, as in the case of carbid, or it may participate catalytically, as in the case where it acts as a solvent for the carbon in

the manner previously referred to. In other words, such claims are to be regarded as of sufficient scope to cover iron, or its equivalent, either as an active participant or as a catalyst. The term "metal of the iron group" used in certain of the claims is intended to cover those metals commonly regarded in analytical work as properly pertaining to the group, *e. g.* manganese, chromium, nickel, cobalt, etc.

Having described my invention, I claim:

1. The process of purifying a metallic mass having impurities therein, one of which comprises carbon, which includes heating said mass and bringing portions, at least, thereof intimately into contact with nitrogenous matter and a powerful reducing element, and effecting a reaction between some of said carbon, nitrogenous matter and reducing element, and also effecting another reaction between some of said reducing element and another of said impurities with which said reducing element is capable of directly uniting.

2. The process of purifying a metallic mass having impurities therein, one of which comprises carbon, which includes heating said mass and bringing portions, at least, thereof intimately into contact with nitrogenous matter and a powerful reducing element, and effecting a reaction between some of said carbon, nitrogenous matter and reducing element, and also effecting another reaction between some of said nitrogenous matter and another of said impurities with which said element is capable of directly uniting.

3. The process of purifying a metallic mass having impurities therein, one of which comprises carbon, which includes heating said mass and bringing portions, at least, thereof intimately into contact with nitrogenous matter and a powerful reducing element, and effecting a reaction between some of said carbon, nitrogenous matter and reducing element, and also effecting another reaction between some of said reducing element and another of said impurities with which said element is capable of directly uniting, and effecting still another reaction between some of said nitrogenous matter and another of said impurities with which nitrogen is capable of directly uniting.

4. The process of purifying a metallic mass having impurities therein, one of which comprises carbon, which includes supplying nitrogenous matter to said mass and effecting a reaction in which the element nitrogen and some of said carbon participate to form cyanogen.

5. The process of purifying a metallic mass having impurities therein, one of which comprises carbon, and one of which comprises an element capable of being united

with nitrogen to form a nitrid, which includes supplying nitrogenous matter to said mass and effecting a plurality of reactions in which the element nitrogen and some of 5 said impurities participate to form nitrogenous compounds, carbon taking part in one of said reactions and yielding cyanogen.

6. The process of purifying a metal which comprises effecting a reaction in which the 10 metal to be treated, a powerful reducing element, the element carbon and a nitrogenous compound participate.

7. The process of treating a mass of material containing carbon in solution in an 15 element normally incapable of directly uniting with free nitrogen, to separate carbon therefrom, which comprises effecting a reaction, at an elevated temperature, in which at least some of said carbon, the element nitrogen, an element capable of acting as the 20 base of a compound containing carbon and nitrogen, and said first mentioned element participate to form said compound, said nitrogen being present previous to said reaction as an element of an inorganic nitrogenous compound.

8. The process of treating a substance containing carbon in solution in an element 30 of the iron group which is capable of directly uniting with free carbon, which comprises combining a portion at least of said carbon with nitrogen to form cyanogen, and with a second element capable of acting as the base of a cyanogen compound, by bringing 35 said second element together with a nitrogenous compound, into intimate contact with said substance, and elevating the temperature of said substance to a point where substantially all of said carbon may be reacted 40 upon by nitrogen obtained in part at least from said nitrogenous compound and by said second element to form said cyanogen compound.

9. The process of treating a mass of material 45 containing carbon in solution in an element normally incapable of directly uniting with free nitrogen, to separate carbon therefrom, which comprises effecting a reaction, at an elevated temperature, in which at least some of said carbon, the element nitrogen, an element capable of acting as the 50 base of a compound containing carbon and nitrogen, and said first mentioned element, participate to form said compound, said nitrogen being present previous to said reaction, as an element of a nitrogenous compound.

10. The process of treating a mass of material 55 containing carbon in solution in an element normally incapable of directly uniting with free nitrogen, to separate carbon therefrom, which comprises effecting a reaction, at an elevated temperature, in which at least some of said carbon, the element ni-

rogen, an element capable of acting as the 65 base of a compound containing carbon and nitrogen in the form of a radical, and said first mentioned element, participate to form said compound, said nitrogen being present, previous to said reaction as an element of a nitrogenous compound.

11. The process of treating a mass of material containing carbon and an element capable of directly uniting with free carbon, but incapable of directly uniting with free 75 nitrogen, to separate carbon therefrom, which comprises effecting a reaction at an elevated temperature, in which at least some of said carbon, the element nitrogen, an initially free element capable of acting as 80 the base of a compound containing carbon and nitrogen, and said first mentioned element, participate to form said compound, said nitrogen being present, previous to said reaction, as an element of a nitrogenous compound.

12. The process of treating a mass of material containing carbon and an element normally incapable of directly uniting with free nitrogen, to separate carbon therefrom, 90 which comprises effecting a reaction at an elevated temperature, in which at least some of said carbon, a mixture of nitrogenous compounds, an element capable of acting as the base of a compound containing carbon 95 and nitrogen, and said first mentioned element, participate to form said compound.

13. The process of treating a mass of material containing carbon in solution in an element capable of directly uniting with free 100 carbon to form a carbid, to separate carbon therefrom, which comprises effecting a reaction, at an elevated temperature, in which at least some of said carbon, a nitrogenous compound, an element capable of 105 acting as the base of a compound containing carbon and nitrogen, and said first mentioned element, participate to form said compound containing carbon and nitrogen, and separating said last mentioned compound from the residue by changing its physical condition.

14. The process of treating a mass of material containing carbon and an element normally incapable of directly uniting with free 115 nitrogen, to separate carbon therefrom, which comprises effecting a reaction at an elevated temperature, in which at least some of said carbon, a nitrogenous compound, an initially free element capable of acting as 120 the base of a compound containing carbon and nitrogen in the form of a radical, and said first mentioned element, participate to form said compound.

15. The process of treating a mass of material 125 containing carbon and iron, to separate carbon therefrom, which comprises effecting a reaction at an elevated temperature

in which at least some of said carbon, the element nitrogen, an initially free element capable of acting as the base of a compound containing carbon and nitrogen in the form of a radical, and iron participate, said nitrogen being present, previous to said reaction, as an element of a nitrogenous compound.

16. The process of treating a mass of material containing carbon and an element of the iron group, to separate carbon therefrom, which comprises effecting a reaction, at an elevated temperature, in which at least some of said carbon, a nitrogenous compound, an initially free element capable of acting as the base of a compound containing carbon and nitrogen in the form of a radical, and said element of the iron group participate.

17. The process of treating a mass of material containing carbon and iron, to separate carbon therefrom, which comprises effecting a reaction at an elevated temperature in which at least some of said carbon, a nitrogenous compound, a light metal capable of acting as the base of a compound containing carbon and nitrogen in the form of a radical, and iron participate.

18. The process of treating a mass of material containing carbon and an element normally incapable of directly uniting with free nitrogen, to separate carbon therefrom, which comprises effecting a reaction at an elevated temperature, in which at least some of said carbon, the element nitrogen, a light metal capable of acting as the base of a compound containing carbon and nitrogen, and said first mentioned element, participate to form said compound, said nitrogen being present, previous to said reaction, as an element of a nitrogenous compound.

19. The process of treating a mass of material containing carbon and an element normally incapable of directly uniting with free nitrogen, to separate carbon therefrom, which comprises effecting a reaction at an elevated temperature, in which at least some of said carbon, the element nitrogen, an alkali metal capable of acting as the base of a compound containing carbon and nitrogen, and said first mentioned element, participate to form said compound, said element nitrogen being present, previous to said reaction, as an element of a nitrogenous compound.

20. The process of treating a mass of material containing iron intimately associated with graphitic carbon whereby to combine portions at least of said carbon with nitrogen, which comprises subjecting said mass of material to heat, bringing a nitrogenous compound and a powerful reducing metal, capable of forming the base of a cyanogen compound which is stable at the temperature of the operation, into intimate contact with said iron and carbon, and effecting a reac-

tion in which portions, at least of said carbon, the nitrogen present in said compound thereof, said powerful reducing metal and said iron participate, to form said cyanogen compound of said reducing metal.

21. The process of treating a mass of material containing iron and carbon whereby to combine portions at least of said carbon with nitrogen, which comprises subjecting said mass of material to heat, bringing a nitrogenous compound and a powerful reducing metal, capable of forming the base of a cyanogen compound which is stable at the temperature of the operation, into intimate contact with said iron and carbon and effecting a reaction in which portions, at least, of said carbon, the nitrogen present in said nitrogenous compound, said powerful reducing metal and said iron participate, to form said cyanogen compound of said reducing metal.

22. The process of purifying a metallic mass having impurities therein, one of which comprises carbon, and one of which comprises an element capable of being directly united with a powerful reducing element, which includes supplying said last mentioned element and the element nitrogen to said mass and effecting a plurality of reactions in which said powerful reducing element and some of said impurities participate to form compounds of said reducing element, carbon taking part in one of said reactions and yielding cyanogen, said nitrogen being supplied to said reaction from a compound thereof.

23. The process of removing impurities from a substance which comprises effecting a reaction in which the substance to be treated, a powerful reducing element, the element carbon, and a compound of nitrogen participate.

24. The process of removing an impurity from a substance which comprises subjecting said substance to contact with a powerful reducing element in vaporous form, and effecting a reaction in which the substance to be treated, said reducing element, the element carbon, and a compound of nitrogen participate.

25. The process of manufacture which includes effecting a reaction at a temperature above 500° C., in which an initially free element capable of being combined with carbon and nitrogen to form a cyanogen compound, stable at the temperature of the operation, the element iron, a nitrogenous compound, and carbonaceous matter in non-gaseous form, participate, substantially as described.

26. The process of manufacture which includes effecting a reaction, through the instrumentality of heat, in which a metal capable of being combined with carbon and nitrogen to form a cyanogen compound,

- stable at the temperature of the operation, a nitrogenous compound, an element of the iron group, and carbonaceous matter in non-gaseous form participate, while substantially excluding water and water forming constituents from participation in said reaction.
27. The process of manufacture which includes effecting a reaction, through the instrumentality of heat, in which a metal capable of being combined with carbon and nitrogen to form a cyanogen compound, stable at the temperature of the operation, a nitrogenous compound, the element iron, and carbonaceous matter in non-gaseous form participate.
28. The process of manufacture which includes effecting a reaction, through the instrumentality of heat, in which metallic sodium, a nitrogenous compound, an element of the iron group and carbon uncombined with oxygen participate, while substantially excluding water and water forming constituents from participation in said reaction.
29. The process of manufacture which includes effecting a reaction, through the instrumentality of heat, in which metallic sodium, a nitrogenous compound, the element iron, and carbon uncombined with oxygen participate.
30. The process of treating a mass of material containing carbon and iron to separate carbon therefrom, which comprises effecting a reaction, at an elevated temperature, in which at least some of said carbon, and inorganic nitrogenous compound, a light metal capable of acting as the base of a compound containing carbon and nitrogen in the form of a radical, and iron participate.
31. The process of manufacture which includes effecting a reaction, through the instrumentality of heat, in which metallic sodium, nitrogen initially present as a constituent of an inorganic compound, the element iron, and carbon participate.
32. The process of manufacture which includes effecting a reaction, through the instrumentality of heat, in which an alkali metal, nitrogen initially present as a constituent of an inorganic compound, the element iron, and carbon participate.
33. The process of manufacture which includes effecting a reaction, through the instrumentality of heat, in which metallic sodium, a nitrogenous compound, the element iron, and carbon participate.

In witness whereof, I subscribe my signature, in the presence of two witnesses.

JOHN E. BUCHER.

Witnesses:  
CHAS. M. PERRY,  
HOWARD C. RIPLEY.